

## UNITED STATES PATENT OFFICE

2,521,438

## GREASE COMPOSITION

John C. Zimmer, Union, and Arnold J. Morway,  
Rahway, N. J., assignors to Standard Oil Development Company, a corporation of Delaware

No Drawing. Application December 6, 1947,  
Serial No. 790,220

6 Claims. (Cl. 252—36)

1

The present invention relates to lubricating greases and more particularly to low temperature lubricating greases which include dibasic acid esters as substantial elements. The present application is a continuation-in-part of application Serial No. 570,784, filed December 30, 1944, now Patent No. 2,436,347, issued February 17, 1948.

In the usual methods of manufacturing low temperature greases, low boiling mineral oil fractions with resultant low flash points and low viscosities are compounded with metallic soaps to form plastic masses, or semi-solid grease compositions. It has been observed that the torque necessary to turn a bearing lubricated by grease is directly proportional to the viscosity of the oil used in the grease at the particular temperature. Therefore, it has been necessary in the manufacture of low temperature greases to use low boiling mineral oil fractions since these fractions have low viscosities at extremely low temperatures ( $-100^{\circ}$  F.). However, since the equipment, for instance the shutter on an aerial reconnaissance camera, on which this grease is to be used may at times be subjected to relatively high temperatures ( $150^{\circ}$  F.), the low boiling mineral oil fractions used in making the grease are limited to those which are not too volatile.

While it is desirable from the standpoint of cost to employ mineral oil fractions as lubricants, their characteristics are not suitable for use under conditions where extreme low temperatures may be encountered and where also fire hazards are present. The use of extremely low boiling mineral oil fractions is feasible in the manufacture of low temperature greases, but such use is subject to drastic restrictions because of the high volatility of such fractions at higher temperatures. In addition, their use creates operational difficulties due to fire hazards encountered in manufacture and use. Also, when the lubricant of volatile characteristics is subjected to high temperatures, loss of the liquid element by evaporation may soon render it deficient for low temperature operations. Hence it is desirable to avoid high volatility without impairing low temperature fluidity.

It has now been found that the esters of aliphatic dibasic acids, particularly those esters in which the esterifying radical is a branched chain alkyl radical, may be used to replace a part of the

2

mineral oil fractions in the production of low temperature greases with improved results. The resulting mixtures, as set forth hereinafter, have excellent lubricating properties at low temperatures, but are not so expensive as the greases claimed in the parent application which employ esters as the entire liquid lubricating element. As stated in the application referred to above, these esters possess unusually high boiling points and resulting low vapor pressures at ordinary room temperatures, high viscosity indices, or low viscosity-temperature coefficient, extremely low pour points and are relatively stable chemically.

Among the aliphatic dicarboxylic acids suitable for the preparation of the esters used in making the grease compositions of the present invention, there may be mentioned malonic, succinic, iso-succinic, glutaric, ethyl malonic, pyro tartaric, adipic, pimelic, suberic, azelaic and sebatic acids. Instead of one of the enumerated acids, any acid or mixture of acids having the formula



where R is a bivalent aliphatic hydrocarbon radical—for example synthetic acids produced by polymerization or dimerization of unsaturated fatty acids or their esters—may be used.

The esters which may be used in making the grease compositions of the present invention have the general formula  $\text{R}_1\text{OOC—R—COOR}_2$ , where R is a bivalent aliphatic hydrocarbon radical such as methylene, polymethylene, ethylidene, propylene, methyl dimethylene, butenylidene and the like;  $\text{R}_1$  and  $\text{R}_2$  are hydrocarbon radicals such as branched chain alkyl, alkaryl and cyclo alkyl radicals of which secondary butyl, benzyl, cyclo hexanol and secondary octyl phenyl are representative. These are generally derived from the corresponding alcohols. Isobutyl 2-ethylhexyl sebacate is an example of a mixed ester. These esters may contain additional constituents or functional groups, such as Cl, Br, NH<sub>2</sub>, NHR, NR<sub>1</sub>R<sub>2</sub>, CHO, CO, SH, SR, RSSR, ROR, ROMetal. The esters may be made by any of the methods for producing esters known to the art.

One suitable method of preparing the esters consists of reacting the alcohol with the acid at elevated temperatures in the presence of an esterification catalyst such as sulfuric acid sulfosalicylic acid, etc. The reaction is facilitated by a continuous removal of water formed during the

reaction by azeotropic distillation with a solvent such as benzene, toluene, etc., or by passing inert gas through the reaction mixture to remove water of reaction. The product is washed with dilute alkali to remove the catalyst and any traces of unreacted acid and, if necessary, is heated under reduced pressure with or without blowing with an inert gas to remove any unreacted alcohol or other low boiling material. If necessary the product can be clay-treated, and it is desirable although not absolutely necessary, that the finished ester have a neutralization number not higher than about 0.2 mg. KOH per gram of ester to obtain suitable stability to oxidation, since free acids left in the finished material can catalyze oxidation of the product, particularly in the presence of materials such as copper or brass at elevated temperatures.

Typical esters together with some of their more significant properties are given in the following table.

—100° F. They meet all of the requirements of Aeronautical Board Specification AN-G-25 for synthetic type low temperature greases. They meet bleeding test requirements in the same specification without difficulty although greases prepared as described above have not been entirely free from a minor degree of ester separation at elevated temperatures.

We have now discovered that greases containing a substantial quantity of mineral lubricating oil, for example 20 to 70% by weight, together with esters as described above in quantities of 80 to 30% of the weight of liquid medium are quite satisfactory and possess certain advantages over lubricants prepared using only the ester. Thus a grease prepared with a liquid base-stock containing 70% by weight of di-2-ethylhexyl sebacate and 30% of mineral lubricating oil, a highly acid treated oil of about 58 S. S. U. at 100° F. derived from naphthenic type crude, passes the copper corrosion test satisfactorily and is superior in the bleeding test to a grease containing

TABLE I

| Name of Ester                      | Centistokes Viscosity at— |         |           | Slope on<br>ASTM Vis-<br>cosity-Temp.<br>Chart for<br>the Interval<br>of 210° F.<br>to —30° F. | Visc.<br>Index | Flash<br>Point | Pour<br>Point,<br>°F. | Approximate<br>Boiling Point,<br>°F. at At-<br>mospheric<br>Pressure |
|------------------------------------|---------------------------|---------|-----------|------------------------------------------------------------------------------------------------|----------------|----------------|-----------------------|----------------------------------------------------------------------|
|                                    | 210° F.                   | 100° F. | —40° F.   |                                                                                                |                |                |                       |                                                                      |
| Di-secondary butyl sebacate        | 2.09                      | 6.42    | 320       | 0.752                                                                                          | 136            | 355            | —90                   | 650                                                                  |
| Di-2-ethylhexyl sebacate           | 3.31                      | 12.64   | 1,532     | 0.707                                                                                          | 152            | 430            | —90                   | 760                                                                  |
| Di-undecanyl sebacate <sup>1</sup> | 4.66                      | 22.83   | 8,000     | 0.716                                                                                          | 138.5          | —              | —85                   | —                                                                    |
| Di-2-ethylhexyl alkylated sebacate | 5.56                      | 42.72   | 2,200,000 | 0.812                                                                                          | 68.5           | —              | —45                   | —                                                                    |
| Di-2-ethylhexyl azelate            | 3.05                      | 11.25   | 1,200     | 0.729                                                                                          | 147            | 410            | —40                   | 750                                                                  |

<sup>1</sup> Alcohol-5 ethyl nonanol 2



<sup>2</sup> Extrapolated from the 100 and 210° F. values.

As disclosed in the parent application referred to above, a suitable low temperature grease composition may comprise di-2-ethylhexyl sebacate and/or di-secondary butyl sebacate, with from 6 to 30% of a soap of a metal selected from the group consisting of alkali and alkaline earth metals together with a stabilizer consisting of an amphoteric metal compound, specifically an oxide, carbonate or soap of zinc or aluminum. As further examples, the composition may consist of a major proportion, for example 65% or more, of di-secondary butyl adipate and di-isopropyl sebacate with 6 to 30% of soap and stabilizer as recited above.

only the ester and the soap. The percentages given above refer to the liquid constituent only and not to the finished grease.

In general, the mineral oil to be used should have a viscosity of 45 to 70 sec. Saybolt at 100° F., a V. I. (viscosity index) of about 50 to 100, a flash point in the range of 275° to 400° F., an A. S. T. M. pour point of about —60 to —30° F. and may be derived from naphthenic or paraffinic type crudes.

The following table gives the complete formulas of two compositions showing comparative properties of greases with and without mineral oil replacing part of the ester.

TABLE II

|            | Composition                   |                    | Penetra-<br>tion<br>(60 Strokes) | 24 hour, 212° F. Cop-<br>per Strip Corrosion | Per cent<br>Bleeding<br>30 hours<br>at 212° F. |
|------------|-------------------------------|--------------------|----------------------------------|----------------------------------------------|------------------------------------------------|
|            | Ingredients                   | Weight<br>Per cent |                                  |                                              |                                                |
| Example I  | Lithium stearate              | 20.0               | 262                              | Pass (No Staining)                           | 3.2                                            |
|            | Phenyl alpha naphthylamine    | 0.5                |                                  |                                              |                                                |
|            | Zinc naphthenate              | 0.5                |                                  |                                              |                                                |
|            | Di-2-Ethyl Hexyl Sebacate     | 79.0               |                                  |                                              |                                                |
| Example II | Hydrogenated fish oil acids   | 17.00              | 261                              | do                                           | 0.6                                            |
|            | Lithium hydroxide monohydrate | 2.88               |                                  |                                              |                                                |
|            | Phenyl alpha naphthylamine    | 0.50               |                                  |                                              |                                                |
|            | Zinc naphthenate              | 0.50               |                                  |                                              |                                                |
|            | Mineral oil 58 SSU at 100° F. | 23.00              |                                  |                                              |                                                |
|            | Di-2-ethylhexyl sebacate      | 56.12              |                                  |                                              |                                                |

The lubricating greases described in the above mentioned application, of which the present is a continuation-in-part, have proved to be very satisfactory for use at temperatures as low as

Table III shows the results obtained upon submission of the greases of Examples I and II to the tests outlined in the Government Specification AN-G-25.

TABLE III

Conformation of experimental greases with test requirements of Government Specification  
AN-G-25

| Tests                                                                                           | AN-G-25 Spec. Requirements     | Example I            | Example II           |
|-------------------------------------------------------------------------------------------------|--------------------------------|----------------------|----------------------|
| Odor                                                                                            | None other than that of ester. | None                 | None.                |
| Homogeneity                                                                                     | Completely homogeneous.        | Homogeneous.         | Homogeneous.         |
| Corrosion on Copper                                                                             | Slight brown stain, only.      | Slight brown stain.  | Pass.                |
| Dropping Point, °F.                                                                             | 325 Minimum.                   | 370                  | 342.                 |
| Worked Penetration at 77° F., mm. m./10.                                                        | 260-300.                       | 262                  | 261.                 |
| Water Resistance at 120° F., Per Cent Washed Out                                                | 20% maximum.                   | 5.0                  | 5.0.                 |
| Low Temperature Torque Test at -67° F., Sec./Rev.                                               | 5 maximum.                     | 2.0                  | 2.8.                 |
| Apparent Viscosity, Poises at -67° F. (20 sec. shear rate)                                      | 15,000 maximum.                | 8000                 | 9.20.                |
| Bleeding, 30 Hours at 212° F. Per Cent Loss                                                     | 5 maximum.                     | 3.2                  | 0.6.                 |
| Evaporation, 20 Hours at 210° F., Per Cent Loss                                                 | 2 maximum.                     | 0.6                  | 1.9.                 |
| Normal Hoffman Bomb Oxidation at 210° F., PSI Pressure Drop in 100 Hours.                       | 5 maximum.                     | 1.0                  | 3.0.                 |
| Storage Stability (4 months at 100-105° F.), Penetration Increase, mm./10.                      | 30 maximum.                    | 10                   | 5.                   |
| Working Stability (100,000 Strokes Fine Hole Plate), Penetration, mm./10.                       | 375 maximum.                   | 316                  | 305.                 |
| Aeration Test (Per Cent Increase in Volume)                                                     | 15 maximum.                    | 4.5                  | 5.0.                 |
| High temperature Performance: No. of Hours run in a ball bearing at 10,000 R. P. M. and 260° F. | 1000 Hours (minimum).          | more than 1000 hours | more than 1000 hours |

The composition containing mineral oil (Example II) was prepared as follows:

The mineral oil and fatty acids were charged to a fire-heated kettle and heated to 150° F. Temperatures of 125° to 200° F. are suitable. The lithium hydroxide, dissolved in boiling water, was added and the acids neutralized and the soap concentrate was dried out at 250° F. while agitating. When the soap concentrate was approximately dry, the temperature was raised to 300° F. and a sample was taken for a free alkalinity determination. The percent free alkali should be in the range of 0.15 to 0.25%, calculated as NaOH. Any adjustments of the free alkali content were made, and thereafter residual water was removed by holding the grease at the elevated temperature of 300° F. The di-2-ethylhexyl sebacate was next added and the temperature was raised further to 400° to 420° F. The phenyl alpha naphthylamine and the zinc naphthenate were then added. The hot molten grease was pumped to a continuous type grease cooler and cooled to 90 to 100° F. in one pass. The finished grease was then ready to be filtered and packaged.

The greases of this invention may be produced in various other ways. For example, the soap may be prepared in situ in the mineral oil by reaction of a fatty material with an alkali or alkaline earth hydroxide, the soap concentrate dried, and the ester then added to the dry oil-soap mixture. Alternatively, the soap may be preformed separately either by direct reaction of a fatty material with an alkali or alkaline earth hydroxide or in the case of lithium, calcium, magnesium or aluminum soaps, by precipitation from water according to well-known procedures. After being dried, the soap may be powdered, if desired, to facilitate dispersion in the ester-mineral oil medium. The soap is then added to the cold ester-oil solution. Once an ester-oil-soap mixture has been obtained, it is heated to a temperature of about 400-450° F. until the soap is completely melted in the liquid ingredients. The molten grease is then cooled either slowly in pans or rapidly in a continuous type grease cooler. The rapid cooling is to be preferred, inasmuch as greases prepared in this manner are more resistant to shear breakdown than those prepared by a slow cooling process. For example, the penetration of a pan-cooled grease rises from 260 mm./10 to 375 mm./10 after only 60 strokes

of an ASTM worker, while a rapidly cooled grease having the same unworked penetration shows a penetration of only 305 mm./10 after 100,000 strokes of the worker. It may be pointed out that in the preparation of the greases of this invention it is not desirable to form the soap in situ in the ester because hydrolysis of the ester occurs and an unsatisfactory product results.

In general, from 4 to 25 parts of fatty material are combined with 1 to 5 parts of saponifying agent, either before or after the fatty material is added to 20 to 40 parts of lubricating oil. After saponification the temperature is raised well above the boiling point of water to dry the soap and thereafter 45 to 65 parts of the ester are added. An oxidation inhibitor, such as 0.01 to 1 part of naphthylamine may be added after the ester. 0.1 to 5 parts of amphoteric metal soap may be added at any stage of the process, preferably after formation of the principal soap.

While lithium hydroxide is the preferred medium, because of the temperature stability properties of lithium soap greases, any of the alkali or alkaline earth metal oxides or hydroxides may be used for neutralizing or saponifying the fatty material. The fatty material may comprise any of the ordinary higher fatty acids, or the fats, or fatty oils, from which they are derived such as stearic acid, oleic, erucic, lauric, palmitic acid, tallow, lard oil, animal fats, etc., may be used to form the soaps with which to make the grease. The saturated acids derived from hydrogenated fish oil are especially suitable. On formulating the greases of the present invention they will contain in general 5 to 30% of alkali or alkaline earth soaps, 65 to 93.5% of the ester-mineral oil mixture or mixture of several esters with mineral oil, and preferably 0.1 to 5% of a stabilizer, preferably an amphoteric metal soap such as zinc or aluminum stearate and related materials. The use of a stabilizer smooths out the texture of the grease and further aids in the actual production of the grease. It is not always essential but is preferably used. The oxides, carbonates, or soaps of metals forming amphoteric oxides such as the soaps of zinc, tin and aluminum, have been found to be very beneficial in their use as stabilizers, particularly in the case of greases containing free alkali. Mixtures of these soaps may also be used, a particularly effective combination being 0.5% aluminum stearate and 0.5% zinc naphthenate.

Greases prepared using a lithium soap and containing mineral lubricating oil of the general character described above in lieu of part of the ester have obvious economic advantages over lubricants of the type described and claimed in the above-mentioned application, Serial No. 570,784.

As described more fully in the above mentioned application, of which the present is a continuation-in-part, there is considerable drag on bearings at low temperatures when ordinary low temperature greases are used. This drag becomes particularly objectionable at extremely low temperatures such as  $-40^{\circ}$  to  $-70^{\circ}$  F. or lower. While very light mineral oils are fairly satisfactory at such low temperatures they evaporate excessively at temperatures of  $120^{\circ}$  to  $150^{\circ}$  F. Such extremes of temperature are commonly encountered in the use of aircraft, and when lubricating greases are subjected to considerable evaporation they are no longer entirely suitable for low temperature lubrication.

Grease compositions comprising substantial quantities of esters of the type described above, in combination with comparable or preferably somewhat smaller quantities of light mineral oils, are not so readily evaporated as those wherein the lubricating fluid consists entirely of a very light hydrocarbon. Somewhat heavier hydrocarbons may be used in combination with esters such as di-2-ethylhexyl sebacate, secondary butyl sebacate and the like without encountering undue torque or drag at very low temperature. By the use of amphoteric metal soap as a stabilizer, excess alkali is absorbed or taken up and thus prevented from reacting with the esters, the composition at the same time retaining the improved oxidation and structural characteristics of the alkaline type greases.

What is claimed is:

1. A low temperature grease composition consisting essentially of 20 to 40% by weight of mineral lubricating oil, 45 to 65% of an ester having the general composition  $\text{COOR}_1(\text{R})\text{COOR}_2$  wherein R is a bivalent aliphatic hydrocarbon radical and  $\text{R}_1$  and  $\text{R}_2$  are branched chain hydrocarbon radicals, 5 to 30% of a soap selected from the group consisting of the alkali and alkaline earth metal soaps, and 0.1 to 5% of amphoteric metal soap as a stabilizer.

2. Composition according to claim 1 in which the amphoteric metal soap stabilizer is a mixture of aluminum stearate and zinc naphthenate.

3. A lubricating grease composition suitable for low temperature use consisting essentially of approximately 56% by weight of di-2-ethylhexyl sebacate, 23% mineral lubricating oil, 19% lithium soap, and less than 1% each of an oxidation inhibitor and an amphoteric metal soap as a stabilizer.

4. Composition according to claim 1 wherein said mineral oil is an oil of 45 to 70 S. S. U. viscosity at  $100^{\circ}$  F., having a flash point of  $275^{\circ}$  to  $400^{\circ}$  F.

5. Process of preparing a low temperature lubricating grease which comprises adding 4 to 25 parts of fatty material to 20 to 40 parts of mineral lubricating oil, heating said fatty material and lubricating oil to  $125^{\circ}$  to  $200^{\circ}$  F., adding 1 to 5 parts of a saponifying agent selected from the class consisting of the alkali and alkaline earth metal oxides and hydroxides, the quantity of saponifying agent used being adjusted to yield a free alkalinity of 0.15 to 0.25, calculated as NaOH, thereafter heating above the boiling point of water to dry the soap, adding 45 to 65 parts of an ester having the general formula  $\text{COOR}_1(\text{R})\text{COOR}_2$  wherein R is a bivalent aliphatic hydrocarbon radical, and  $\text{R}_1$  and  $\text{R}_2$  are branched chain hydrocarbon radicals, and adding a small amount of an amphoteric metal soap to take up excess alkali and stabilize the grease.

6. Process according to claim 5 wherein 0 to 1 part of an oxidation inhibitor and 0.1 to 5 parts of an amphoteric metal soap are added during processing.

JOHN C. ZIMMER.  
ARNOLD J. MORWAY.

#### REFERENCES CITED

The following references are of record in the file of this patent:

#### UNITED STATES PATENTS

| Number       | Name           | Date           |
|--------------|----------------|----------------|
| 2,363,013    | Morway et al.  | Nov. 21, 1944  |
| 2,383,147    | Morgan         | Aug. 21, 1945  |
| 45 2,391,113 | Zimmer et al.  | Dec. 18, 1945  |
| 2,436,347    | Zimmer et al.  | Feb. 17, 1948  |
| 2,448,567    | Zisman et al.  | Sept. 7, 1948  |
| 2,450,221    | Ashburn et al. | Sept. 28, 1948 |
| 2,450,222    | Ashburn et al. | Sept. 28, 1948 |